

(No Model.)

N. WASHBURN.

CAR WHEEL.

No. 356,907.

Patented Feb. 1, 1887.

Fig. 1.



Fig. 2.



Fig. 3.



Fig. 4.



Witnesses.

S. N. Piper.

18.13. Finey

Inventor.

Nathan Washburn.

by R. H. Eddy atty.

# UNITED STATES PATENT OFFICE.

NATHAN WASHBURN, OF ALLSTON, MASSACHUSETTS.

## CAR-WHEEL.

SPECIFICATION forming part of Letters Patent No. 356,907, dated February 1, 1887.

Application filed November 1, 1886. Serial No. 217,688. (No model.)

*To all whom it may concern:*

Be it known that I, NATHAN WASHBURN, of Allston, in the county of Suffolk, of the Commonwealth of Massachusetts, have invented a new and useful Improvement in the Manufacture of Railway-Car Wheels; and I do hereby declare the same to be described in the following specification, and represented in the accompanying drawings, of which—

15 Figure 1 is a transverse and median section, and Fig. 2 a side elevation, of a car wheel embodying my invention, the nature of which is defined in the claims hereinafter presented. Fig. 3 is a side view, and Fig. 4 is an end view, 15 of its hub-thimble or perforated wrought-iron tube.

This wheel, with the exception of part of its hub, is made of "manganese steel," the remaining part of the hub consisting not only of an 20 interlining of cast-iron united with the steel in the process of casting, or a thin wrought or cast iron tube having numerous transverse perforations or holes in it, but of a tubular interlining of cast-iron cast within the tube and, 25 when such tube is perforated, extending through its holes, and welded or united to both tube and the mass of metal surrounding such tube.

In Figs. 1 and 2 of the drawings the body of the wheel of manganese steel is shown at A, 30 the perforated iron tube at B, and the cast-iron tubular lining at C, they being disposed concentrically with each other, as represented.

In the process of making this wheel the thin metallic tube B, having numerous holes through it laterally, is laid in the matrix or mold for casting the wheel so as to be concentric with the circumference of the mold, after which a 35 cylindrical core of a less diameter than that of the bore of the said tube B is to be placed concentrically within such tube, both tube and core being firmly fixed in position. Next the manganese steel to constitute the wheel-body is to be cast into the mold, and at the same time or immediately after a quantity of melted 40 cast-iron sufficient to fill the space between the core and the perforated tube, and also the perforations of such tube, is to be run into such space, so as to fill it and the said perforations and unite with the metal surrounding 45 the tube.

As soon or soon after the metal may have

become set in the mold, the whole wheel or casting in its highly-heated state is to be removed therefrom and plunged into a bath of cool water or into a cistern thereof, into which 55 water in a cool state may be continuously running and from which it at top may be escaping at a higher temperature. In such cistern or water the wheel is to be allowed to remain until it may become cool or sufficiently 60 acted upon by the water. By so applying water to the manganese-steel wheel the latter becomes greatly toughened or strengthened.

The manganese steel is a combination of metallic manganese and wrought-iron melted in 65 a crucible with a suitable flux, the product being low in carbon, the manganese generally varying from six to twenty per cent. of the composition. In preparing this steel I usually melt the wrought-iron and the manganese 70 in separate crucibles rather than in one, and just before casting the metal, or while it is in the ladle, the melted manganese is to be poured into and thoroughly incorporated with it.

For a method of preparing "metallic manganese" and what is known in the arts as "manganese steel," reference may be had to the British Patent No. 1,660 for 1857.

Were that part of the hub of the wheel in which the eye is formed for reception of an 80 axle to be of manganese steel, it, owing to the hardness of such metal, could not easily be bored or reamed to the proper diameter; but by making such part of a tubular mass of cast-iron united, as described, to the mass of manganese steel such eye can easily be enlarged 85 and finished as may be required.

I claim, as an improved manufacture—

1. A car-wheel having its body of manganese steel and part of the hub in which the 90 eye is situated of cast-iron, and between such part and body and concentric, or about so, therewith a perforated iron tube, the mass of cast-iron being united through the perforations of the tube with the mass of manganese 95 steel.

2. A car-wheel having its body of manganese steel and the part of the hub in which the eye is situated of cast-iron, and the whole or the manganese-steel part toughened or strengthened by being immediately, after becoming of 100 sufficient hardness to be removed from the

mold in which the wheel may have been founded, subjected to the action of a bath of cold water, as set forth.

3. A car-wheel having its body of manganese steel and part of the hub in which the eye is situated of cast-iron, and between such part and body and concentric, or about so, therewith a perforated iron tube, the mass of cast-iron being united through the perforations of the tube with the mass of manganese

steel, and the whole or the manganese-steel part toughened or strengthened by being immediately, after becoming sufficiently indurated to be removed from the mold in which the wheel may have been founded, subjected to the action of a bath of cold water, as set forth.

NATHAN WASHBURN.

Witnesses:

R. H. EDDY,  
R. B. TORREY.